

Patented Sept. 7, 1926.

## UNITED STATES PATENT OFFICE.

HORACE JAMES HEGAN, OF COVENTRY, ENGLAND, ASSIGNOR TO COURTAULDS  
LIMITED, OF LONDON, ENGLAND.MANUFACTURE AND PRODUCTION OF THREADS, FILAMENTS, STRIPS, OR FILMS  
FROM CELLULOSE COMPOUNDS.

No Drawing. Application filed January 13, 1925, Serial No. 2,178, and in Great Britain February 2, 1924.

This invention consists in an improved manufacture and production of threads, filaments, strips, or films, by precipitating, or coagulating, cellulose esters from solutions thereof.

According to this invention a solution of a cellulose ester, (such, for example, as cellulose acetate) in any suitable solvent, or mixture of solvents, is projected through 10 suitably shaped orifices, or otherwise introduced into a fatty acid such as can be obtained from animal, or vegetable, oils, or fats, oleic acid being particularly suitable for the purposes of this invention. A single 15 fatty acid of the kind aforesaid, or a mixture of such acids, can be employed as may be desired. The cellulose compound, in the process according to this invention, is rapidly precipitated and can be freed from any 20 excess of acid in any suitable manner.

In this way, artificial silk of good quality can be spun, and products of great pliability and freedom from blemishes be obtained.

The cellulose ester employed may be dissolved in any suitable solvent, or solvents, miscible with the acid, or acids, used for precipitating and these solvents can be readily and completely recovered from the acid, or acids, by distillation, or by any other suitable means.

If desired, an animal oil, or a vegetable oil such for instance as castor oil, linseed oil, or cod-liver oil (or more than one such oil) can be used in admixture with the aforesaid fatty acid or fatty acids.

The following is an example of a manner in which this invention can be performed but I do not limit myself to this example.

Dissolve cellulose acetate in four times its 40 weight of acetone and project the solution through a jet containing eighteen holes each of one-tenth of a millimetre diameter into a bath of oleic acid, maintained at a temperature of, or about, 35 degrees centigrade. 45 The acetone is removed from the cellulose

acetate leaving this latter in the form of a thread, composed of eighteen filaments. This thread is led through a sufficient extent of the bath to coagulate the said thread which is then wound onto a bobbin. The 50 excess of oleic acid can be subsequently removed by means of any suitable solvent (such as a dilute alkali), or by centrifugal action.

The foregoing example can be varied by 55 replacing the acetone, partly or wholly, by any other suitable solvent, for instance, a mixture of acetone and ethyl-alcohol can be employed. Also, if desired, an animal, or vegetable, oil can be mixed with the oleic 60 acid; for instance the coagulating bath may be composed of two parts of oleic acid, and one part each of castor oil and olive oil.

In the following claims the expression "fatty acid" is to be read as meaning a fatty 65 acid such as can be obtained from animal, or vegetable, oils, or fats, and mixtures of such acids; and the expression "an oil" includes castor-oil, linseed oil, cod-liver oil, and other animal, or vegetable, oils and mixtures of such oils.

## What I claim is:—

1. The manufacture of threads, filaments, strips and films, by projecting a solution of cellulose ester into a coagulating bath containing 75 a fatty acid such as can be obtained from animal, or vegetable, oils, or fats.

2. The manufacture of threads, filaments, strips and films, from a solution of cellulose acetate in acetone by projecting such solution into a bath containing oleic acid.

3. The manufacture of filaments, threads, strips and films from a solution of cellulose acetate in acetone, by projecting such a solution into a bath containing oleic acid and 85 an oil.

In testimony whereof I have signed my name to this specification.

HORACE JAMES HEGAN.